

May 15, 1934.

R. CROSS  
ANTIKNOCK COMPOUND FOR INTERNAL COMBUSTION  
ENGINES AND PROCESS OF MAKING SAME  
Original Filed Dec. 1, 1924

1,958,744

*Fig. 1.*



*Fig. 2.*



*Fig. 3.*



INVENTOR.  
Roy Cross

BY *Thos. E. Scofield.*

ATTORNEY.

## UNITED STATES PATENT OFFICE

1,958,744

## ANTIKNOCK COMPOUND FOR INTERNAL COMBUSTION ENGINES AND PROCESS OF MAKING SAME

Roy Cross, Kansas City, Mo.

Original application December 1, 1924, Serial No. 753,069. Divided and this application February 17, 1932, Serial No. 593,530

3 Claims. (Cl. 44—9)

This invention relates to improvements in anti-knock compounds or "anti-pinking" compounds to be mixed with motor fuel to prevent and eliminate the so-called knock from gasoline engines.

5 This factor in the operation of gasoline engines is especially prevalent when the motor is working under a heavy load with an advanced spark. Considerable work has been done upon the elimination of this objectionable feature of internal combustion engines, and it has been found that the addition of certain compounds or minerals soluble in the motor fuel will retard the knocking in the motor.

10 This application is a divisional application of my application Serial No. 753,069, filed December 1, 1924.

15 It has been found that certain organic compounds free from mineral matter and halogens and containing from 20% to 80% nitrogen have a very effective retarding action on the force of the explosion if combined and mixed with the explosive gas or mixture of hydrocarbon and air used as fuel. Generally, it may be said that the greater the amount of nitrogen and carbon present, the more valuable the anti-knock properties; or in other words, the smaller the amount of hydrogen the more valuable the anti-knock property.

20 The most valuable specific compounds for this purpose are: cyanamide,  $(CN-NH_2)$ ; dicyanamide,  $(CN-NH_2)_2$ ; urea,  $CO(NH_2)_2$ ; cyan-anilid,  $CN-NH-C_6H_5$ ; cyanic acid,  $CONH$ ; hydrazine,  $N_2H_4$ .

25 The most valuable of these compounds is cyanamide because of its exceptional anti-detonating effect, its high percentage of nitrogen, its distillation temperature and its solubility in ether and hydrocarbon oils. The dicyanamide is equally effective, but is very difficult to incorporate with motor fuels as it is practically insoluble in ether and is only soluble in alcohol to the extent of substantially 1.25%. Anhydrous ammonia  $NH_3$  used in conjunction with dicyanamide in some instances has given very satisfactory results—the ammonia in addition to the dicyanamide, having certain anti-knock properties when mixed with gasoline.

30 When using cyanamide, the amount necessary to give the desired results, will vary according to the character and detonating proclivities of the oil treated. Amounts varying from 0.1% to 1.0%, depending upon the fuel, have been effectively used. The particular value of this class of compounds, in addition to their anti-detonating properties, lies in their cheapness and the fact that

they do not contain any metallic or mineral substances and that they do not produce any poisonous substances in the engine exhaust or cause injury to the metal parts. In addition to this, dicyanamide is, at the present time, produced on a large scale and in large quantities without danger to those engaged in its manufacture. The substance from which cyanamide is obtained is usually calcium cyanamide which, at the present time, has a value of about 3¢ per pound.

35 The effect of anti-knock substances can be readily determined by mounting a gasoline engine upon a block and fitting thereto a suitable indicator card registering the character of the explosion by means of a curve which shows upon the indicator card the operation of the motor on the various fuel mixtures which are used.

In the drawing:

40 Fig. 1 shows the operation of the motor upon gasoline marketed at a nearby filling station and is characteristic of the present day motor fuel. The sharp angular curves coming to a decided peak, shows the presence of engine knock or pinging.

45 Fig. 2 shows a curve made with the same fuel with the addition of 0.1% of cyanamide. The curve is noticeably smoother than either of the foregoing, and brings out the effectiveness of this material as an anti-detonating compound.

50 Fig. 3 shows a curve made with the addition of 3% of carbon tetrachloride. In this case the knocking properties are even more pronounced than in the curve shown in Fig. 1.

55 In each case, the curve was registered on the indicator card when the motor operation was substantially identical as to load and timing of the spark.

60 A suitable method of preparing anti-knock motor fuel from the compounds mentioned is to make a concentrated solution of cyanamide, cyanoform, cyan-anilid, urea or other nitrogenous compounds, in ether, benzol, gasoline or similar solvent. This concentrated solution is then added to the gasoline in the necessary quantity to attain the desired effect. As mentioned, certain 65 motor fuels require more anti-detonating material than others. For example, the California oils are notoriously anti-detonating in their effect, as is benzol and other fuels. On the other hand, certain oils from particular wells have 70 the characteristic of knocking very easily when used as a motor fuel and must be mixed with a compound of this character—especially when used in an engine having high compression or one 75 fouled with carbon deposition.

From the curve shown in the drawing, it will be noted that cyanamide and aniline seem to have the strongest anti-detonating properties. The effectiveness of cyanamide is probably due, in part, to the fact that it has a very low heat of combustion. This slowing of the explosion allows the fuel to be burned a little more completely and reduces the amount of carbon monoxide discharged through the exhaust. By this 10 consumption or conversion of carbon monoxide to carbon dioxide, more power is obtained, and by the slowing of the explosion, the carbon knock is eliminated.

A further advantage of cyanamide, and some 15 of the nitrogenous compounds mentioned, is that they volatilize at a temperature below the end-point and approximating the average distillation temperature of ordinary motor fuel or gasoline. Thus, there is no deposition or accumulation 20 of objectionable carbon in the engine cylin-

ders. They also normally have a considerable vapor tension at ordinary temperature.

The percentage of nitrogenous compounds, as specified in the claims, is shown or approximated by the chemical formulae.

Having thus described my invention, what I claim is:

1. A motor fuel for internal combustion engines comprising in combination a hydrocarbon of gasoline-like nature and a small quantity of a compound selected from the following group: cyanamide, cyanic acid, cyan-anilid, dicyan-diamide, urea, hydrazine.

2. A hydrocarbon motor fuel for internal combustion engines containing a small amount of dissolved cyanamide.

3. A hydrocarbon motor fuel for internal combustion engines containing a small amount of dissolved cyan-anilid.

ROY CROSS. 95

25 100

30 105

35 110

40 115

45 120

50 125

55 130

60 135

65 140

70 145

75 150